

# UNITED STATES PATENT OFFICE.

MAX BIELEFELDT, OF BERLIN, GERMANY.

## NITROGLYCERIN EXPLOSIVE.

No. 799,705.

Specification of Letters Patent.

Patented Sept. 19, 1905.

Application filed March 21, 1905. Serial No. 251,324.

*To all whom it may concern:*

Be it known that I, MAX BIELEFELDT, a subject of the German Emperor, residing at Berlin, Germany, have invented certain new and useful Improvements Relating to Nitroglycerin Explosives, of which the following is a specification.

The present invention has for its object to render explosives containing nitroglycerin as far as possible uncongealable or to avoid their liability to freeze at low temperatures. For this purpose dinitro-monochlorhydrin is added to the explosives, the quantity used being fifteen to twenty-five per cent. of the weight of nitroglycerin contained in the same.

The improved compositions may be obtained either by adding to the explosives pure dinitro-chlorhydrin or by using for the manufacture of explosives nitroglycerin containing dinitro-chlorhydrin.

In comparison with the addition of dinitro-glycerin to the explosives for the same purpose the addition of dinitro-chlorhydrin offers the following advantages: Dinitro-chlorhydrin may be produced easily, free from danger and efficiently as regards the quantity ob-

tainable in practice in comparison with the theoretical yield; it does not lower the temperature at which the explosion takes place and is not liable to decomposition; it prevents 30 the freezing of dynamite better than any other substance hitherto used for this purpose—for instance, dinitro-glycerin—and it accelerates the gelatinizing process of the explosives.

What I claim is—

1. A nitroglycerin explosive containing dinitro-monochlorhydrin, to protect the explosive from the danger of freezing, substantially as described.

2. A nitroglycerin explosive containing dinitro-monochlorhydrin, between fifteen and twenty-five per cent. of the weight of nitroglycerin contained in the explosive, substantially as described.

In testimony whereof I have hereunto set my hand in presence of two subscribing witnesses.

MAX BIELEFELDT.

Witnesses:

FRDR. LUTZE,  
A. KREFT.